

HOXSIE & REED.

Flexible Tubing.

No 44,425.

Patented Sept. 27, 1864.



Fig. 2.



Witnesses:

Paul A. Brundt  
Samuel Bassett

Inventor:

David Hoxsie  
Thomas L. Reed

# UNITED STATES PATENT OFFICE.

DAVID K. HOXSIE AND THOMAS L. REED, OF PROVIDENCE, R. I.

## IMPROVED FLEXIBLE TUBE OR HOSE.

Specification forming part of Letters Patent No. 44,425, dated September 27, 1864.

*To all whom it may concern:*

Be it known that we, DAVID K. HOXSIE and THOMAS L. REED, both of Providence, in the county of Providence and State of Rhode Island, have invented a new and useful Improvement in Flexible Tubing or Hose for the Conveyance of Gas, Water, &c.; and we do hereby declare the following specification to be a full, clear, and exact description of the same, reference being had to the accompanying drawings, making part of such specification, in which—

Figure 1 represents a section of our improved tubing or hose; and Fig. 2 represents an improved apparatus which is designed to be used in the application of our improvement to tubing, hose, &c.

Our improvement consists in the use of animal intestines properly prepared and applied as an impervious sheath or covering in the formation of flexible tubing or hose.

Considerable difficulty has hitherto been experienced in making an article of flexible tubing that would be impervious, particularly to illuminating-gas, for the reason that the naphtha which is deposited by condensation from such gas softens and dissolves india-rubber (caoutchouc) and such gums, glutinous materials, and compounds as have been heretofore employed in the manufacture of tubing to make it impervious, and this difficulty, it is believed, is effectually removed by the improved sheath or covering mentioned.

To enable others skilled in the art to make and use our invention, we will proceed to describe the same.

In Fig. 1 of the said drawings, A represents a section of tubing which is formed of a spiral wire coil, over which is a covering of braided cotton, which is stuffed and covered with black enamel varnish to render the cotton covering impervious to gas. This enamel varnish soon softens and dissolves by the action of the naphtha before referred to and causes the tube to leak gas, and in order to prevent such leakage we draw over the said coating of varnish one or more intestines, one over the other, each being moist and supple when it is drawn upon the tube, and each being allowed to dry before drawing on another. In drying, the intestines shrink snugly and smoothly upon the surface of the tubing and upon each other, and furnish an impervious sheath or covering to the same. The best intestines for this purpose are those of lambs, which are of about the right size and

free from kernels and other imperfections. The intestines are prepared by removing the refuse matter, washing clean, and, if not needed for immediate use, they may be packed in fine dry salt. A solution composed of one pound of alum, one half pound of salt, dissolved in two quarts of water, in which the intestines are to be soaked, will cleanse them and give them additional strength.

The intestines may, however, be more perfectly prepared or cured by the following solution: Peruvian bark, one ounce; oak bark, one ounce; wormwood, one ounce; gentian root, one ounce; tobacco, one ounce; water, two pounds.

Steep the ingredients in the water and add one ounce of alum to the solution. After the intestines have been properly cleansed they may be placed in this solution and there remain until required for use.

As a convenience for drawing the intestines upon the tubing the metal tube G, Fig. 2, may be used, the intestines being taken from the solution and drawn upon the said tube, when, by passing the tubing A through the tube G and seizing both the intestine and the protruding end of the tubing with the hand, the latter is drawn through the tube, drawing the intestine from the exterior of said tube upon the tubing.

It is better to use two or three layers or coverings of intestines, one over the other, so that in case one of the coverings is punctured it may be covered and protected by succeeding ones.

The intestines may be covered to form a finish by braiding thereon cotton, silk, or worsted, or this braided covering may be varnished or stuffed with boiled linseed-oil to form a finished coating, or otherwise, as may be desired.

The intestinal covering is designed to be used as an impervious sheath in combination with any and all compositions of materials forming a tube or hose.

Having described our invention and the manner of preparing and applying the same, what we claim, and desire to secure by Letters Patent, is—

The use of animal intestines as an impervious covering for tubing or hose, as described.

DAVID K. HOXSIE,  
THOMAS L. REED.

Witnesses:

ISAAC A. BROWNELL,  
SAMUEL BARRATT.